

## UNITED STATES PATENT OFFICE

2,163,553

## EXPANSION JOINT MATERIAL

Albert C. Fischer, Chicago, Ill., assignor to The Philip Carey Manufacturing Company, a corporation of Ohio

No Drawing. Application January 31, 1934,  
Serial No. 709,187

4 Claims. (Cl. 106—31)

In the art it has been the practice to use ordinary asphaltic or bituminous materials in the preparation of expansion joints, and in many of these cases, finely divided, saturated fibrous material. Asphalts of various kinds, except at a very low melting point and very high penetration, at 32° F. become very brittle in winter, and the shock often breaks this material, leaving the joint in a manner to destroy its efficiency.

10 This invention relates to a treatment of the bituminous material with a polymerized oil, in order to add to the life of the asphalt or bituminous material and at the same time make the material more elastic. This may be accomplished by 15 introducing in the bituminous material any oil which will polymerize readily at a high heat. As one example, typifying a suitable oil, China-wood oil sets to a jelly-like mass when heated to about 500° F. and is suitable for carrying out the invention. By retarding the heating, this mass may be 20 produced in a stringy consistency.

This case is a continuation in part of application Serial No. 76,904, (Patent No. 1,982,506) filed December 21, 1925.

25 The salient feature of my invention consists in either mixing polymerized oil with the asphalt or else mixing unpolymerized oil with the asphalt and subjecting the mixture to a temperature sufficient to polymerize the oil in the mix. By varying the temperature above the degree necessary to 30 polymerize the oil I am enabled to obtain various results.

This combination of materials may be effected by polymerized China-wood oil, employing varying proportions of the polymerized oil, one formula being five (5) per cent polymerized oil and ninety-five (95) per cent of suitable bituminous material, or varying proportions, increasing the proportion of polymerized oil and decreasing the 40 proportion of bituminous material, depending upon the consistency of the mass desired. Where it is desirable to incorporate any of the fibrous material mentioned, percentages varying from three to twenty-five per cent may be readily incorporated with mechanical mixers, known to the art. A combination of materials which has been found to produce a satisfactory expansion joint 45 consists in a mixture of five (5) per cent polymerized China-wood oil, eighty-five (85) per cent bituminous material and ten (10) per cent finely divided material.

The invention is not limited to the China-wood oil, as any oil, whether of mineral, vegetable or

animal origin, which polymerizes is suitable. Among other suitable oils, cotton seed oil, linseed oil, soya bean oil, cedar, castor oil, cocoanut oil, rape oil, neat's-foot oil, corn oil, perilla oil, lard oil, fish oil (Menhaden, etc.), mutton fat, stearic acid, oleic acid, and the like, are enumerated as further specific examples. Stearin pitch and cotton seed oil pitch may also be considered as products containing various proportions of polymerized oils and which would therefore be suitable for the purpose intended.

By the addition of dryers in the oil, or the use of sulphur, the polymerization may be somewhat hastened.

While I have described one preferred embodiment of the invention and enumerated other specific examples of a suitable oil, or the like, it will be understood that such details are for the purpose of illustration and not a limitation of the invention.

Neither do I wish to be limited to the fibrous matter mentioned, as many other types of fibrous matter may be suitable. Also finely divided matter may be employed, if it is desirable that the entire mass be waterproofed. The resulting product is one of an elastic nature and one which will prolong the life of the asphalt or bituminous material, and at the same time strengthen the binding material resulting from the mixture.

After mixing this material, as outlined, in any suitable mechanical mixer, it may be presented to pressing rolls, also previously known to the art, suitable for reducing the batch to flat sheets, then cutting said sheets into strips, adapting the material for use as premoulded expansion joints.

I claim:

1. A premoulded expansion joint consisting of a mixture of five (5) per cent polymerized cotton-seed oil, eighty-five (85) per cent bituminous material and ten (10) per cent finely divided material.

2. A premoulded expansion joint comprising a mixture of polymerized cotton-seed oil, bituminous material and finely divided filling material.

3. Expansion joint material comprising a mixture of polymerized cotton-seed oil and bituminous material.

4. Expansion joint material comprising a mixture of polymerized cotton-seed oil and bituminous material, said oil having the character of having been polymerized at high heat and set to a jelly-like consistency.

ALBERT C. FISCHER.